

W.C. Joy & J. Campbell.

Paper Bleaching Mach.

No 87,779.

Patented Mar. 16, 1869.



Fig. 2.



Witnesses;

S S Pepled

Geo C Hanfman

Inventor;

Wm C Joy

John Campbell



WILLIAM C. JOY AND JOHN CAMPBELL, OF PENN YAN, NEW YORK.

Letters Patent No. 87,779, dated March 16, 1869.

IMPROVEMENT IN PREPARING AND BLEACHING PAPER-PULP.

The Schedule referred to in these Letters Patent and making part of the same.

To all whom it may concern:

Be it known that we, WILLIAM C. JOY and JOHN CAMPBELL, of Penn Yan, in the county of Yates, and State of New York, have invented a new and useful Improvement in Preparing and Bleaching Paper-Pulp and fibrous materials; and we do hereby declare that the following is a full, clear, and exact description of the construction and operation of the same, reference being had to the annexed drawings, making a part of this specification, in which—

Figure 1 is a longitudinal vertical section.

Figure 2 is a bird's-eye view.

The letters of reference refer to the same parts in each figure.

The nature of our invention consists in making and using an apparatus, and applying chemical agents to bleach paper-pulp and other material, so as to accomplish, with our improvement, the following results, viz:

First, the efficacious change and removal of all coloring-matter, without injuring the fibre or destroying it, and at the same time freeing the pulp or material of all used agents.

Second, disintegrating the fibre while bleaching, without macerating it.

To enable others skilled in the art to make and use our invention, we will proceed to describe its mode of construction and operation.

A is the base on which the various parts are placed, and is identical with the floor of the bleaching-room.

B is a rotary fan, used to force a powerful current of air through the pipe C into the bleaching-engine. An air-pump of sufficient capacity may be used in its stead, if preferred. This fan may be actuated by a belt from any convenient power. It drives a powerful current of air through the pipe C, into the lower part of the bleaching-engine, as represented in the figure. It also drives a current of air through the gas-generator that carries the proper quantity of gas, to facilitate the bleaching. It must be placed higher than the engine, or the pipe C must be deflected upward, to prevent the agents or materials rising into the fan.

C is a pipe extending from the fan to the engine. It enters the engine, near its bottom, as shown in fig. 1. Its use is to convey air into the engine, and discharge the same at the bottom of the mass being bleached. The end of the pipe must be directed in the course that the material is moved while passing around in the engine, so that its force will assist the motion of the material, and allow a greater quantity to be bleached at the same time. This pipe has the induction-pipe of the gas-generator united with it, as shown in the figures.

D is the gas-generator. It must be made of lead, or other material that will be least corroded by action of the chemicals. Its shape is represented in fig. 1. It is placed into and is supported by a reservoir that will hold water. The reservoir may be provided with pipes for hot water or steam, to heat the generator, as re-

quired. The generator is provided with a cover, that has a rim, or flanch, at the under side, that fits into a channel that surrounds the top of the generator. The cover may be fastened if its own weight is not sufficient. The channel is then filled with water to lute the joint, to prevent gas escaping. The generator is provided with an agitator, as shown in fig. 1, to mix and agitate the chemicals, and it has a pipe at the bottom, for discharging sediment, and cleaning it, as shown in fig. 2. It is also provided with an induction-pipe, E, and education-pipe, F, as shown in each figure.

E is the induction-pipe. It is connected with the pipe C, and extends into the generator. It is provided with a stop-cock, to regulate the quantity of air, or stop it, from the generator.

F is the education-pipe leading from the generator to the engine, as shown in the figures. It is provided with a stop-cock, to regulate or stop the passage of gas through it. This pipe extends into the engine, and the end is bent downward, as shown in fig. 1. The use of this pipe is to convey the gas into the engine, and discharge it when the current of air is operating upon the material, thus producing the ozone modification, oxygen, and using it for bleaching at the time it is generated.

G is the bleaching-engine. It is made in shape like the ordinary beating-engine, and is represented in the figures, or any other form or shape of vessel may be used if preferred.

It is best to have the vessel provided with a cover, made in sections, so that the material may readily be put into it. That portion of the cover immediately above the induction, air, and gas-pipes must be securely fastened, to prevent the material from escaping.

One part of the cover may have an exhaust-pipe, I, to carry off the waste and spent gas, and discharge it out of the bleaching-room.

A chlorine solution is put into the engine, of less strength than is used for bleaching in the ordinary way. The material to be bleached is then put in, and the cylinder of the engine is put in motion, for the purpose of stirring the mass. A current of air, at any temperature, is introduced by the pipe C at the same time, and a stream of gas is also introduced simultaneously with the air and stirring.

By these operations the ozone modification of oxygen is brought, at the instant it is created, in almost immediate contact with the whole of the material being bleached.

When the bleaching is accomplished, the gas is shut off, and, by the continuous use of air, and stirring, the material is freed from chlorine before hydrochloric acid is formed to the injury of the material; and by the conjoint action of these agencies, the disintegration of fibre is more easily and perfectly accomplished, a longer fibre produced, with less waste of material by maceration, and the destruction of fine particles of fibre by the action of hydrochloric acid avoided.

H is a stirring-cylinder, with plain paddles, that will carry the material and solution over the backfall, thus giving motion to the mass.

I is a discharge-pipe, for conducting air, gas, and vapor from the engine out of the bleaching-room. It must be made large enough to allow the escape of all the air and gas forced into the engine, and all gas and vapor arising from the chlorine solution.

If the air, gas, and vapor, are not injurious in the bleaching-room, a portion of the cover may be opened or removed, so that there will be no resistance to their escape, which will allow the air and gas from the pipes C and F to perform their functions with less resistance, and allow ozone a free agency in changing and removing the coloring-matter.

Having thus fully described our invention,

What we claim as new, and desire to secure by Letters Patent, is—

1. The construction and application of the generator D, when used as and for the purpose set forth.

2. Producing the ozone modification of oxygen, by applying a powerful current of air, in combination with chlorine, to an aqueous solution containing the material to be bleached, while the mass is being agitated.

3. The arrangement of the fan B and engine G, when applied and used as and for the purpose specified.

4. The use of a current of air, for the purpose of removing chlorine from fibrous materials after the process of bleaching, in the manner substantially as set forth.

5. Preventing the formation of hydrochloric acid in the mass or solution, by accomplishing the bleaching, and removing the chlorine, also preventing the destruction of the fine particles of fibre, or the hardening of any portion thereof, by the means and in the manner specified.

6. Disintegrating fibrous materials by the use of a powerful current of air forced into or among the same, while the material is being operated upon by any bleaching-agent in an open vessel, as herein described.

7. The use of a current of air to assist in giving rapid circulation to the material while being bleached.

8. The free discharge of the air, gas, and vapor from the bleaching-engine, substantially as and for the purpose set forth.

WM. C. JOY.  
JOHN CAMPBELL.

Witnesses:

S. S. RAPLEE,  
GEO. C. KAUFMANN.